# EUROPEAN PATENT APPLICATION

(11) **EP 4 745 672 A1**
(43) Date of publication of application: **20.05.2026**
(21) Application number: 25214843.2
(22) Date of filing: 11.11.2025
(51) Int. Cl.: G03G 9/107, G03G 9/113

(54) **MAGNETIC CARRIER AND TWO COMPONENT DEVELOPER CONTAINING THE SAME, AND METHOD FOR PRODUCING MAGNETIC CARRIER**

(30) Priority: 14.11.2024 JP 2024199255
(71) Applicant: KYOCERA Document Solutions Inc., Osaka-shi, Osaka 540-8585 (JP)
(72) Inventor: SAKAMOTO, Noriaki, Osaka-shi, Osaka, 540-8585 (JP)
(74) Representative: Heuer, Wilhelm

(57) **Abstract**

Magnetic carrier includes a carrier core (1) and a resin coat layer (5) that coats the surface of the carrier core (1) and can electrostatically charge toner by friction. The carrier core (1) has, in a depressed part (3) in its surface, fine particles (4) of which the volume average primary particle size is 1 µm or less. The amount of fine particles (4) present on the surface of the carrier core (1) is, on a number basis when the particle distribution of the carrier core (1) is measured, 2% or more but 20% or less.

## Description

### BACKGROUND

The present disclosure relates to magnetic carrier that electrostatically charges toner by friction, to two-component developer containing magnetic carrier, and to a method for producing magnetic carrier.

In general, in electrophotography, the surface of an electrostatic latent image carrying member is electrostatically charged by corona discharge or the like and is then exposed to laser light or the like to form an electrostatic latent image. The formed electrostatic latent image is developed with toner to form a toner image. The formed toner image is then transferred to a recording medium to obtain a high-quality image. Known methods for developing an electrostatic latent image include: two-component development, which uses, as developer, two-component developer containing toner and magnetic carrier; one-component development, which uses, as developer, one-component developer containing no magnetic carrier; and the like. For higher image quality and faster printing, two-component development is suitably used.

Two-component developer used in two-component development contains magnetic carrier and toner, of which only the toner is consumed in development and the carrier is repeatedly used while being stirred in a development device. To cope with increasingly high durability desired nowadays, as carrier particles, use is made of resin-coated magnetic particles (coating carrier) in which the surface of the magnetic particle (carrier core) is coated with a resin layer (coat layer).

The conventional method for producing coating carrier, in which the coat layer is not sufficiently fixed to the surface of the carrier core, can cause the peeling-off of the coat layer in durability printing. In addition, a thin part partly present in the coat layer, or an insufficient amount of resin with which to coat can result in the carrier having poor durability (life span). Also, carrier with low roundness and hence insufficient fluidity mixes insufficiently with toner, and this leads to insufficient charging of toner.

### SUMMARY

An object of the present disclosure is to provide magnetic carrier for use in electrophotography that excels in charging ability and charge keeping ability even in a high-temperature high-humidity environment and that permits development with high durability and high image quality, to provide two-component developer containing such magnetic carrier, and to provide a method for producing such magnetic carrier.

According to one aspect of the present disclosure, magnetic carrier includes a carrier core and a resin coat layer that coats the surface of the carrier core and can electrostatically charge toner by friction. The carrier core has, in a depressed part in its surface, fine particles of which the volume average primary particle size is 1 µm or less. The amount of fine particles present on the surface of the carrier core is, on a number basis when the particle distribution of the carrier core is measured, 2% or more but 20% or less.

### BRIEF DESCRIPTION OF THE DRAWINGS

Fig. 1 is a sectional view showing a carrier core 1 before smoothing.
Fig. 2 is a sectional view showing the carrier core 1 after smoothing.
Fig. 3 is an enlarged sectional view around the surface of the carrier core 1 after smoothing shown in Fig. 2.
Fig. 4 is an enlarged sectional view around the surface of the carrier core 1, showing a state with a resin coat layer 5 formed on the carrier core 1 after smoothing.
Fig. 5 is an electron microscope photograph at a 500 times magnification of carrier core C-1 used in a practical example.
Fig. 6 is an electron microscope photograph at 1000 times magnification of carrier core C-1 used in the practical example.
Fig. 7 is an electron microscope photograph at 500 times magnification of carrier core C-4 used in the practical example.
Fig. 8 is an electron microscope photograph at 1000 times magnification of carrier core C-4 used in the practical example.
Fig. 9 is an electron microscope photograph at 500 times magnification of carrier core C-6 used in the practical example.
Fig. 10 is an electron microscope photograph at 1000 times magnification of carrier core C-6 used in the practical example.

### DETAILED DESCRIPTION

An embodiment of the present disclosure will be described in detail below. Unless otherwise defined, a result of evaluation (i.e., a value related to a shape, property, or the like) with respect to a powdery substance (specifically, toner core particle, toner base particle, external additive, toner, and the like) is given as a number average of values obtained by measuring respectively for an appropriate number of average particles selected from the powdery substance. Unless otherwise defined, a number average particle size of a powdery substance is a number average value of the circle-equivalent diameter (the diameter of a circle with the same area as the projection area of a particle) of primary particles measured under a microscope. Unless otherwise defined, a measured value of the volume median diameter (D50) of a powdery substance is a value measured using a laser diffraction/scattering particle size distribution analyzer ("LA-750" produced by HORIBA, Ltd.). Unless otherwise defined, a measured value of an acid number or a hydroxy group number is a value measured in conformity with JIS (Japanese Industrial Standards) K0070-1992. Unless otherwise defined, a measured value of a number average molecular weight (Mn) or a mass average molecular weight (Mw) is a value measured by gel permeation chromatography.

In the following description, "-based" is occasionally appended to the name of a compound to collectively refer to that substance and their derivatives. Whenever the name of a compound has "-based" appended to it to refer to the name of a polymer, the repeating unit in the polymer is derived from any of that compound and their derivatives. The term "(meth)acrylic" is occasionally used to refer to "acrylic" and "methacrylic" collectively. The term "(meth)acryloyl" is occasionally used to refer to "acryloyl" (CH₂=CH-CO-) and "methacryloyl" (CH₂=C(CH₃)-CO-) collectively.

The magnetic carrier according to the present disclosure is a powdery substance composed of a plurality of carrier particles (each a particle configured as described later). Moreover, the carrier particle according to the present disclosure has a carrier core and a resin layer coating the carrier core. To produce a carrier particle, the carrier core can be formed of a magnetic material (e.g., ferrite).

The magnetic carrier according to the present disclosure electrostatically charges positively chargeable toner positively, for example, by friction. It along with the positively chargeable toner constitutes two-component developer, which can be used suitably for the development of an electrostatic latent image. To form a high-quality image, the amount of toner in two-component developer is preferably 5 parts by mass or more but 15 parts by mass or less for 100 parts by mass of carrier. Note that positively chargeable toner is electrostatically charged positively by friction with carrier.

The magnetic carrier according to the embodiment can be used to form an image, for example, on an electrophotographic apparatus (image forming apparatus). One example of an image forming method on an electrophotographic apparatus will be described below.

First, based on image data, an electrostatic latent image is formed on a photosensitive member (e.g., a superficial part of a photosensitive drum). Next, the formed electrostatic latent image is developed with two-component developer containing toner and carrier. In the development process, toner (e.g., toner electrostatically charged positively by friction with the carrier) on a development sleeve (e.g., a superficial part of a development roller in the developing device) disposed near the photosensitive member is attached to the electrostatic latent image to form a toner image on the photosensitive member. In the subsequent transfer process, the toner image on the photosensitive member is directly transferred to a recording medium (e.g., sheet); or it is primarily transferred to an intermediate transfer member (e.g., a transfer belt) and then the toner image on the intermediate transfer member is secondarily transferred to the recording medium. Then, the toner is heated to fix the toner to the recording medium. As a result, an image is formed on the recording medium. By superposing on each other toner images of four colors, for example, black, yellow, magenta, and cyan, it is possible to form a full-color image.

### [1. Basic Configuration of Magnetic Carrier]

The magnetic carrier according to the embodiment has a basic configuration as described below. The magnetic carrier includes a plurality of carrier particles each including a magnetic carrier core and a resin coat layer (coat layer). The resin coat layer coats the surface of the magnetic carrier core. The resin coat layer can coat the entire surface of the magnetic carrier core or can partly coat the surface of the magnetic carrier core.

The carrier core has, in a depressed part in its surface, fine particles of which the volume average primary particle size (D50) is 1 µm or less. The presence of the fine particles in the depressed part of the carrier core helps achieve coating in a way that the resin that forms the resin coat layer filtrates through the fine particles to enter the depressed part. This helps the coat layer to be firmly fixed to the carrier core. In addition, the presence of the fine particles leads to an increased surface area of the carrier and thus leads to an increased amount of resin that forms the resin coat layer. This improves the durability of the carrier.

Moreover, the fine particles filling the depressed part of the carrier core serve to flatten the irregularities on the surface of the carrier core. This improves the roundness of the carrier core. Forming the resin coat layer on this carrier core further improves the roundness and improves the fluidity of the carrier. Thus, by forming an image using the magnetic carrier with the above-described basic configuration, it is possible to obtain an excellent charging ability and charge keeping ability in a high-temperature high-humidity environment and to form an image with high image quality over a long period of time.

### [2. Basic Configuration of Toner]

The magnetic carrier according to the embodiment can be blended with toner for use as two-component developer. As toner used with the magnetic carrier, any known positively chargeable toner for two-component developer can be used.

Toner includes a plurality of toner particles each having a toner core particle. The toner core particle at least contains a binder resin, a release agent, and a colorant. The toner core particle can have its surface coated with a shell layer. The shell layer preferably coats 50% or more but 99% or less of the area of a surface region of the toner core particle. The toner core particle can have its entire surface coated with the shell layer. If the toner core particle is coated with a shell layer, the particle composed of the toner core particle and the shell layer is referred to as a toner base particle. If the toner core particle is coated with no shell layer, the toner core particle alone is referred to as a toner base particle.

The thickness of the shell layer can be measured by observing a section of the toner using a transmission electron microscope (TEM) and analyzing the TEM image using a commercially available image analysis software. Usable as commercially available image analysis software are "WinROOF" (developed by MITANI CORPORATION) and the like. How the shell layer coats the surface of the toner can be checked using a scanning electron microscope (SEM). How the shell layer is formed or the inside of the shell layer can be checked by observing a section of the toner using a transmission electron microscope (TEM).

The toner base particle can have an external additive attached to its surface. As the external additive, inorganic fine particles or resin fine particles can be used. Attaching resin fine particles as the external additive to the toner base particle tends to improve the cleaning properties (e.g., adhesion resistance against the photosensitive drum) of the toner as well as its development properties (e.g., transferring efficiency). This is considered to be because, with the resin fine particles functioning as a spacer, the toner less tends to attach to the photosensitive drum, an intermediate transfer belt, or the like.

### [3. Material and Production Method of Magnetic Carrier]

Next, components that are essential or optional for the magnetic carrier according to the present disclosure will be described. The magnetic carrier according to the present disclosure at least includes a carrier core and a resin layer. The resin layer can contain a conductive agent as needed. Now, a description will be given one by one of the carrier core that forms the magnetic carrier particle, the resin material that forms the resin layer, the conductive agent, and a method of producing the magnetic carrier according to the present disclosure.

### (Carrier Core)

The carrier core is not particularly limited and any known carrier for electrophotography employing a two-component system can be used. Examples include: ferrite or magnetite; metal such as iron, nickel, and cobalt; an alloy or a mixture of any of the metals and the like just mentioned with a metal such as copper, zinc, antimony, aluminum, lead, tin, bismuth, beryllium, manganese, magnesium, selenium, tungsten, zirconium, vanadium; a mixture of any of ferrite and the like just mentioned with a metal oxide such as iron oxide, titanium oxide, and magnesium oxide, a nitride such as chrome nitride and vanadium nitride, or a carbide such as silicon carbide and tungsten carbide; and ferromagnetic ferrite. Particularly preferred are ferrite and magnetite.

The volume average particle size of the carrier core is preferably 20 µm or more but 100 µm or less, and more preferably 30 µm or more but 65 µm or less. A carrier core with an average particle size less than 20 µm exhibits low magnetization per particle and causes carrier development. A carrier core with an average particle size larger than 100 µm leads to a reduced specific surface area for contact with toner and hence a low toner charging ability and causes toner scattering. In addition, the concentration of toner in the developer (the mass ratio of toner to carrier, T/C) cannot be set high and thus, inconveniently, satisfactory development properties cannot be achieved. The volume average particle size can be measured using a laser diffraction/scattering particle size tester. Usable as a laser diffraction/scattering particle size tester is, for example, LA-700 (manufactured by HORIBA, Ltd.).

### (Resin Material)

Usable as the resin forming the resin coat layer is silicone-based resin. Silicone-based resin is a resin having a polysiloxane structure (e.g., alkyl polysiloxane structure). Examples of silicone-based resins include silicone resins having a methyl group and epoxy resin-modified silicone resins. Examples of silicone resins having a methyl group include silicone resins having a methyl group but no phenyl group and silicone resins having a methyl group and a phenyl group (hereinafter, occasionally referred to as "methyl phenyl silicone resins"). Preferable as the silicone-based resin are methyl phenyl silicone resins or epoxy resin-modified silicone resins. Examples of silicone-based resin include "SR-2411" (manufactured by Toray Dow Corning Corp.).

Instead of silicone-based resin, polyimide silicone resin, which excels in toner filming properties and durability and which has low water vapor permeability, can be used. Polyimide silicone resin has a polyimide structure and a polysiloxane structure (e.g., alkyl polysiloxane structure). Examples of polyimide silicone resins include "KJR-651," "KJR-655," "KJR-657," and "KJR-663" (all manufactured by Shin-Etsu Chemical Co., Ltd.). Polyimide silicone resin can be a resin obtained by setting a thermosetting polyimide silicone resin.

Also usable is a mixture of polyimide silicone resin as described above and fluorine-containing resin, which excels in toner filming properties and in charging ability with positively chargeable toner. Preferred as the fluorine-containing resin is one or more resins selected from the group consisting of polyvinyl fluoride, polyvinylidene fluoride, tetrafluoroethylene-hexafluoropropylene copolymer (FEP), polytrifluoroethylene (more specifically, polychlorotrifluoroethylene and the like), polyhexafluoropropylene, tetrafluoroethylene-perfluoroalkyl vinyl ether copolymer (PFA), and polytetrafluoroethylene (PTFE). Particularly preferred are FEP, PFA, and PTFE. The mixing ratio of polyimide silicone resin to fluorine resin is preferably 1:9 to 9:1 by mass, and more preferably 2:8 to 8:2.

### (Conductive Agent)

Preferably the resin coat layer additionally contains a conductive agent. The resin coat layer additionally containing a conductive agent allows adjustment of the electric resistance of the carrier particle and its toner charging ability.

Examples of the conductive agent include carbon black (in particular, conductive carbon black), metal oxide particles (e.g., titanium oxide particles and tin oxide particles), and organic conductive agents. As the conductive agent, carbon black or titanium oxide particles are preferred.

If the resin coat layer contains carbon black, the amount of carbon black contained is preferably, for 100 parts by mass of the coating resin, 1.0 parts by mass or more but 10.0 parts by mass or less, and more preferably 2.0 parts by mass or more but 6.0 parts by mass or less.

### (Additives)

The resin coat layer can contain as an additive at least one of a charge control agent, an adhesion improving agent, and a cross-linking agent. As the additive, a silane coupling agent (or a component derived from a silane coupling agent) is preferred and an aminosilane coupling agent (or a component derived from an aminosilane coupling agent) is more preferred. An aminosilane coupling agent (or a component derived from an aminosilane coupling agent) has the functions of a charge control agent, an adhesion improving agent, and a cross-linking agent.

If the resin coat layer contains an additive, the amount of additive contained is preferably, for 100 parts by mass of the coating resin, 4.0 parts by mass or more but 20.0 parts by mass or less, and more preferably 8.0 parts by mass or more but 15.0 parts by mass or less.

### (Production Method for Magnetic Carrier)

One example of a production method for the carrier according to the present disclosure will be described. The production method for the carrier includes a smoothing step where the surface of the carrier core is ground and a depressed part in the surface of the carrier core is filled with a fine powder, an application step where a resin coat layer forming solution is applied to the carrier core, and a heating step where the carrier core after the application step is heated. The resin coat layer forming solution contains a coating resin such as silicone-based resin, a solvent, and other components (e.g., a conductive agent and an additive) that are added as needed.

Examples of the solvent for the resin coat layer forming solution include lactam compounds (e.g., 2-pyrrolidone and N-methyl-2-pyrrolidone), ketone compounds (e.g., methyl ethyl ketone and methyl isobutyl ketone), cyclic ether compounds (e.g., tetrahydrofuran and tetrahydropyran), alcohol compounds (e.g., normal butanol and isobutanol), ester solvents (e.g., ethyl acetate and isobutyl acetate), and aromatic hydrocarbon compounds (e.g., toluene and xylene). Preferred as the solvent for the resin coat layer forming solution is N-methyl-2-pyrrolidone. Preferably, the resin coat layer forming solution has a solid content concentration of 3% by mass or more but 20% by mass or less.

### (Smoothing Step)

In this step, carrier cores are stirred using a mixer to grind off elevated parts on the surface of the carrier core to smoothen it. Figs. 1 and 2 are the sectional views of a carrier core 1 before and after smoothing, respectively. As shown in Fig. 1, in the carrier core 1 before smoothing, its surface has elevated parts 2 and depressed parts 3. The elevated parts 2 have sharp points. On the other hand, as shown in Fig. 2, in the carrier core 1 after smoothing, the elevated parts 2 have their points ground to be rounded.

Fig. 3 is an enlarged sectional view around the surface of the carrier core 1 after smoothing shown in Fig. 2. Through the smoothing step involving the griding of the elevated parts 2, fine particles 4 are generated that contains the same components as the carrier core 1. The fine particles 4 have a volume average primary particle size of 1 µm or less and, as shown in Fig. 3, they concentrate and deposit in the depressed parts 3 of the carrier core 1.

That is, through the smoothing step, the elevated parts 2 of the carrier core 1 are ground to be rounded and the fine particles 4 resulting from the elevated parts 2 being ground fill the depressed parts 3 of the carrier core 1. This enhances the roundness of the carrier core 1. Moreover, since the fine particles 4 results from the elevated parts 2 of the carrier core 1 being ground off, they do not adversely affect the physical properties of the carrier core 1. Furthermore, there is no need for separately adding fine particles for filling the depressed parts 3 and this contributes to reducing the manufacturing cost.

The amount of fine particles 4 present on the surface of the carrier core 1 is preferably such that, on a number basis, the amount of fine particles 4 of 1 µm or less present is preferably 2% or more but 20 % or less.

Usable as the mixer in the smoothing step is, for example, a multipurpose mixer (manufactured by NIPPON COKE & ENGINEERING CO., LTD.). The amount of fine particles 4 on the carrier core 1 can be adjusted by controlling the rotation rate and stirring time of the mixer in the smoothing step.

### (Application Step)

Examples of methods of applying the resin coat layer forming solution to the carrier core include immersing the carrier core in the resin coat layer forming solution and spraying the carrier core in a fluidized bed with the resin coat layer forming solution. In the method where the carrier core is immersed in the resin coat layer forming solution, to elevated parts of the surface of the carrier core, a small amount of resin coat layer forming solution is applied and, to depressed parts of the surface of the carrier core, a large amount of resin coat layer forming solution is applied; thus the resin coat layer forming solution tends to be applied in uneven amounts.

In contrast, in the method where the resin coat layer forming solution is sprayed to the carrier core in the fluidized bed, the resin coat layer forming solution tends to be applied evenly to both elevated and depressed parts of the surface of the carrier core. Thus, preferred as the method of applying the resin coat layer forming solution to the carrier core is spraying the resin coat layer forming solution to the carrier core in the fluidized bed.

In the present disclosure, the carrier core 1 is subjected to the smoothing step, so that the carrier core 1 has enhanced roundness. Thus, it is possible to apply the resin coat layer forming solution to the surface of the carrier core 1 in even amounts as compared with a case where the smoothing step is not performed.

### (Heating Step)

In this step, the carrier core after the application step is heated to remove the solvent contained in the resin coat layer forming solution. If the resin coat layer forming solution contains unset polyimide silicone resin, the unset polyimide silicone resin is set by the heat. As a result, a resin coat layer is formed from the resin coat layer forming solution. The heating can be performed under the conditions of, for example, a heating temperature of 200°C or more but 300°C or less and a heating time of 30 minutes or more but 90 minutes or less.

Fig. 4 is an enlarged sectional view around the surface of the carrier core 1, showing a state where a resin coat layer 5 is formed on the carrier core 1 after smoothing. The carrier core 1 after the smoothing step has enhanced roundness. This permits the resin coat layer forming solution to be applied while keeping an even layer thickness of the resin coat layer 5 between the elevated part 2 and depressed part 3 in the carrier core 1. In addition, the coating proceeds such that the resin coat layer forming solution filtrates through the fine particles 4 deposited in the depressed part 3. This brings about an anchoring effect that achieves firmer fixing of the resin coat layer 5 to the carrier core 1.

### [4. Materials of and Production Method for Toner]

Next, essential or optional components of the toner to be mixed with the magnetic carrier according to the present disclosure will be described. The toner core particle at least contains, in the binder resin, a release agent and a colorant. The toner core particle can also contain a charge control agent, a magnetic powder, and the like as needed. The toner according to the present disclosure can have, if desired, its surface treated with an external additive.

A description will be given below, one by one, of the binder resin, the release agent, the charge control agent, the colorant, and the magnetic powder that form the toner core particle, a shell material for cases where a shell layer is formed, the external additive, and a method of producing the toner according to the present disclosure.

### (Binder Resin)

The toner core particle that forms toner contains a binder resin. The binder resin that can be contained in the toner core particle is not particularly limited so long as it is a resin that is known to be used as a binder resin in toner. Specific examples of the binder resin include thermoplastic resins such as styrene-based resins, acrylic-based resins, styrene-acrylic-based resins, polyethylene-based resins, polypropylene-based resins, vinyl chloride-based resins, polyester resins, polyamide resins, polyurethane resins, polyvinyl alcohol-based resins, vinyl ether-based resins, N-vinyl-based resins, and styrene-butadiene resins. Among these resins, in terms of the dispersion properties of the colorant in the binder resin, the charging properties of the toner, and the fixing properties on sheets, a polyester resin is preferred. The polyester resin will be described below.

Usable as polyester resins are those obtained by condensation polymerization or condensation copolymerization of a dihydric or a trihydric or higher alcohol component and a divalent or a trivalent or higher carboxylic acid component. Examples of components used to synthesize a polyester resin include alcohol components or carboxylic acid components as mentioned below.

Specific examples of dihydric or trihydric or higher alcohol components include: diols such as ethylene glycol, diethylene glycol, triethylene glycol, 1,2-propylene glycol, 1,3-propylene glycol, 1,4-butanediol, neopentyl glycol, 1,4-butenediol, 1,5-pentanediol, 1,6-hexanediol, 1,4-cyclohexanedimethanol, dipropylene glycol, polyethylene glycol, polypropylene glycol, and polytetramethylene glycol; bisphenols such as bisphenol A, hydrogenated bisphenol A, polyoxyethylene bisphenol A, and polyoxypropylene bisphenol A; and trihydric or higher alcohols such as sorbitol, 1,2,3,6-hexanetetrol, 1,4-sorbitan, pentaerythritol, dipentaerythritol, tripentaerythritol, 1,2,4-butanetriol, 1,2,5-pentanetriol, glycerol, diglycerol, 2-methylpropanetriol, 2-methyl-1,2,4-butanetriol, trimethylolethane, trimethylolpropane, and 1,3,5-trihydroxymethylbenzene.

Specific examples of divalent or trivalent or higher carboxylic acid components include divalent carboxylic acids such as maleic acid, fumaric acid, citraconic acid, itaconic acid, glutaconic acid, phthalic acid, isophthalic acid, terephthalic acid, cyclohexane dicarboxylic acid, succinic acid, adipic acid, sebatic acid, azelaic acid, and malonic acid, and alkyl or alkenyl succinic acids such as n-butyl succinic acid, n-butenyl succinic acid, isobutyl succinic acid, isobutenyl succinic acid, n-octyl succinic acid, n-octenyl succinic acid, n-dodecyl succinic acid, n-dodecenyl succinic acid, isododecyl succinic acid, and isododecenyl succinic acid; and trivalent or higher carboxylic acids such as, 1,2,4-benzenetricarboxylic acid (trimellitic acid), 1,2,5-benzene tricarboxylic acid, 2,5,7-naphthalene tricarboxylic acid, 1,2,4-naphthalene tricarboxylic acid, 1,2,4-butanetricarboxylic acid, 1,2,5-hexanetricarboxylic acid, 1,3-dicarboxyl-2-methyl-2-methylenecarboxypropane, 1,2,4-cyclohexane tricarboxylic acid, tetra (methylene carboxyl) methane, 1,2,7,8-octane tetracarboxylic acid, pyromellitic acid, and empole trimer acid. These divalent or trivalent or higher carboxylic acid components may be used as ester-forming derivatives such as acid halides, acid anhydrides, and lower alkyl esters. Here, the term "lower alkyl" denotes an alkyl group with one to six carbon atoms.

When the binder resin is a polyester resin, the softening point of the polyester resin is preferably 70°C or more but 130°C or less, and more preferably 80°C or more but 120°C or less. For improved mechanical strength of the toner core particle and improved fixing properties of the toner, the number average molecular weight (Mn) of the polyester resin is preferably 1000 or more but 2000 or less. The molecular weight distribution of the polyester resin (the ratio Mw / Mn of mass average molecular weight (Mw) to number average molecular weight (Mn)) is preferably 9 or more but 21 or less.

As the binder resin, it is preferable to use a thermoplastic resin for its satisfactory fixing properties on sheets. Here, a thermoplastic resin can be used not only singly but also with a cross-linking agent or a thermosetting resin added to it. Adding a cross-linking agent or a thermosetting resin so that the binder resin partly has a cross-linked structure helps improve the heat-resistant preservation properties, durability, and the like of the toner without degrading the fixing properties of the toner. When a thermosetting resin is used, the cross-linked fraction (gel fraction) of the binder resin extracted using a Soxhlet extractor is, with respect to the mass of the binder resin, preferably 10 mass% or less, and more preferably 0.1 mass% or more but 10 mass% or less.

As a thermosetting resin usable with a thermoplastic resin, an epoxy resin or a cyanate-based resin is preferred. Examples of suitable thermosetting resins include bisphenol A-type epoxy resins, hydrogenated bisphenol A-type epoxy resins, novolak-type epoxy resins, polyalkylene ether-type epoxy resins, cyclic aliphatic group-type epoxy resins, and cyanate resins. Two or more of these thermosetting resins can be used in combination.

The glass transition point (Tg) of the binder resin is preferably 40°C or more but 70°C or less. If the glass transition point is too high, the fixing properties of the toner at a low temperature tends to be poor. If the glass transition point is too low, the heat-resistant preservation properties of the toner tends to be poor.

The glass transition point of the binder resin can be determined from the changing point of the specific heat of the binder resin using a differential scanning calorimeter (DSC). More specifically, the glass transition point of the binder resin can be determined by plotting the endothermic curve of the binder resin using a differential scanning calorimeter (DSC-6200, manufactured by Seiko Instruments Inc.), as a measuring instrument. 10 mg of a measurement sample is put in an aluminum pan while an empty aluminum pan is used as a reference. From the endothermic curve of the binder resin plotted through measurement in a normal-temperature normal-humidity environment in the range of measurement temperature from 25°C or more but 200°C or less at a heating rate of 10°C per minute, the glass transition point of the binder resin can be determined.

The mass average molecular weight (Mw) of the binder resin is not particularly limited within the scope consistent with the object of the present disclosure. Typically, the mass average molecular weight (Mw) of the binder resin is preferably 20,000 or more but 300,000 or less, and more preferably 30,000 or more but 200,000 or less. The mass average molecular weight of the binder resin can be determined by gel permeation chromatography (GPC) using a standard curve previously prepared using a standard polystyrene resin.

### (Colorant)

The toner core particle contains a colorant. As the colorant that can be contained in the toner core particle, any known pigment or dye that suits the color of the toner can be used. Specific examples of colorants that can be suitably added to the toner include: black pigments such as carbon black, acetylene black, lamp black, aniline black; yellow pigments such as chrome yellow, zinc yellow, cadmium yellow, yellow iron oxide, mineral fast yellow, nickel titanium yellow, Naples yellow, naphthol yellow S, Hansa yellow G, Hansa yellow 10G, benzidine yellow G, benzidine yellow GR, quinoline yellow lake, permanent yellow NCG, tartrazine lake, monoazo yellow, and diazo yellow; orange pigments such as reddish chrome yellow, molybdenum orange, permanent orange GTR, pyrazolone orange, Vulcan Orange, and indanthrene brilliant orange GK; red pigments such as red iron oxide, cadmium red, red lead, mercury cadmium sulfide, permanent red 4R, lithol red, pyrazolone red, Watchung red calcium salt, lake red D, brilliant carmine 6B, eosine lake, rhodamine lake B, alizarin lake, brilliant carmine 3B, and monoazo red; violet pigments such as manganese violet, fast violet B, and methyl violet lake; blue pigments such as Prussian blue, cobalt blue, alkali blue lake, partially chlorinated Victoria blue, fast sky blue, indanthrene blue BC, and phthalocyanine blue; green pigments such as chrome green, chromium oxide, pigment green B, malachite green lake, and final yellow green G; white pigments such as zinc white, titanium oxide, antimony white, and zinc sulfide; and extender pigments such as barite powder, barium carbonate, clay, silica, white carbon, talc, and alumina white. Two or more of these colorants can be used in combination for the purpose of adjusting the toner to the desired hue and the like.

The amount of colorant used is not particularly limited within the scope consistent with the object of the present disclosure. Specifically, the amount of colorant used is, relative to the total mass of the toner core particle, preferably 1 mass% or more but 10 mass% or less, and more preferably 2 mass% or more but 7 mass% or less.

A colorant can be used as a master batch having a colorant previously dispersed in a resin material such as a thermoplastic resin. When a colorant is used as a master batch, the resin contained in the master batch is preferably a resin of the same type as the binder resin.

### (Release Agent)

For the purpose of improving its fixing properties and offset resistance, the toner core particle can contain a release agent. The type of release agent that can be contained in the toner core particle is not particularly limited within the scope consistent with the object of the present disclosure. As the release agent, wax is preferred. Examples of wax include carnauba wax, synthetic ester wax, polyethylene wax, polypropylene wax, fluorocarbon resin-based wax, Fischer-Tropsch wax, paraffin wax, montan wax, and rice wax. Two or more of these release agents can be used in combination. Adding these release agents to the toner core particle helps more efficiently suppress offsetting and image smearing (stain around an image caused by its being rubbed).

When a polyester resin is used as the binder resin, from the viewpoint of compatibility, as a release agent, one or more release agents selected from the group consisting of carnauba wax, synthetic ester wax, and polyethylene wax is suitably used. On the other hand, when a polystyrene-based resin is used as the binder resin, likewise from the viewpoint of compatibility, as a release agent, Fischer-Tropsch wax and/or paraffine wax is suitably used.

Fischer-Tropsch wax is a straight-chain hydrocarbon compound with few iso-structure molecules or side-chains that is produced by exploiting the Fischer-Tropsch reaction, which is a catalytic hydrogenation reaction of carbon monoxide.

Preferred among different types of Fischer-Tropsch wax are those that have a mass average molecular weight of 1,000 or more of which the bottom temperature of the endothermic peak observed by DSC measurement falls within the range of 100°C or more but 120°C or less. Examples of such types of Fischer-Tropsch wax include the following products available from Sasol Ltd.: Sasol Wax C1 (endothermic peak bottom temperature: 106.5°C), Sasol Wax C105 (endothermic peak bottom temperature: 102.1°C), Sasol Wax Spray (endothermic peak bottom temperature: 102.1°C), and the like.

The amount of release agent used is not particularly limited within the scope consistent with the object of the present disclosure. Specifically, the amount of release agent used is, relative to the total mass of the toner core particle, preferably 1 mass% or more but 10 mass% or less. Using too small an amount of release agent can result in less-than-expected suppression of offsetting or image smearing in image formation; using too large an amount of release agent can result in fusing-together of toner particle and hence poor heat-resistant preservation properties of toner.

### (Charge Control Agent)

The toner core particle can contain a charge control agent for the purposes of improving the charge level of the toner and the charge response properties as the index of whether it can be charged to a predetermined charge level in a short time, and thereby obtaining toner with excellent durability and stability. Since the magnetic carrier according to the embodiment is used in development with the toner positively charged, a positively chargeable charge control agent is used.

The type of charge control agent that can be contained in the toner core particle is not particularly limited within the scope consistent with the object of the present disclosure. Any of charge control agents known to be used in toner can be appropriately selected and used. Specific examples of positively chargeable charge control agents include: azine compounds such as pyridazine, pyrimidine, pyrazine, orthoxazine, metaoxazine, paraoxiazine, orthothiazine, metathiazine, parathiazine, 1,2,3-triazine, 1,2,4-triazine, 1,3,5-triazine, 1,2,4-oxadiazine, 1,3,4-oxadiazine, 1,2,6-oxadiazine, 1,3,4-thiadiazine, 1,3,5-thiadiazine, 1,2,3,4-tetrazine, 1,2,4,5-tetrazine, 1,2,3,5-tetrazine, 1,2,4,6-oxatriazine, 1,3,4,5-oxatriazine, phthalazine, quinazoline, and quinoxaline; direct dyes composed of azine compounds, such as azine fast red FC, azine fast red 12BK, azine violet BO, azine brown 3G, azine light brown GR, azine dark green BH/C, azine deep black EW, and azine deep black 3RL; nigrosine compounds, such as nigrosine, nigrosine salts, and nigrosine derivatives; acid dyes composed of nigrosine compounds, such as nigrosine BK, nigrosine NB, and nigrosine Z; metal salts of naphthenic acid or higher fatty acids; alkoxylated amines; alkylamides; and quaternary ammonium salts, such as benzylmethylhexyldecylammonium and decyltrimethylammonium chloride. Among these positively chargeable charge control agents, nigrosine compounds are particularly preferred for their faster charge response properties. Two or more of these positively chargeable charge control agents can be used in combination.

Also usable as a positively chargeable charge control agent are resins that have as a functional group a quaternary ammonium salt, a carboxylic acid salt, or a carboxyl group. More specific examples include: styrene-based resins having a quaternary ammonium salt, acrylic-based resins having a quaternary ammonium salt, styrene-acrylic-based resins having a quaternary ammonium salt, polyester resins having a quaternary ammonium salt, styrene-based resins having a carboxylic acid salt, acrylic-based resins having a carboxylic acid salt, styrene-acrylic-based resins having a carboxylic acid salt, polyester resins having a carboxylic acid salt, styrene-based resins having a carboxylic group, acrylic-based resins having a carboxylic group, styrene-acrylic-based resins having a carboxylic group, and polyester resins having a carboxylic group. The molecular weight of these resins are not particularly limited within the scope consistent with the object of the present disclosure, and they can be in the form of an oligomer or a polymer.

Among resins usable as a positively chargeable charge control agent, from the viewpoint of easy adjustment of the amount of charge within a desired range, styrene-acrylic-based resin having as a functional group a quaternary ammonium salt is more preferred. Specific examples of preferred acrylic-based comonomers for copolymerization with the styrene unit in styrene-acrylic-based resin having as a functional group a quaternary ammonium salt include esters of alkyl (meth)acrylates such as methyl acrylate, ethyl acrylate, n-propyl acrylate, iso-propyl acrylate, n-butyl acrylate, iso-butyl acrylate, 2-ethylhexyl acrylate, methyl methacrylate, ethyl methacrylate, n-butyl methacrylate, and iso-butyl methacrylate.

Used as a quaternary ammonium salt is a unit derived by a quaternization process from a dialkyl aminoalkyl (meth)acrylate, dialkyl (meth)acryl amide, or dialkyl aminoalkyl (meth)acryl amide. Specific examples of dialkyl aminoalkyl (meth)acrylate include dimethylaminoethyl (meth)acrylate, diethyl aminoethyl (meth)acrylate, dipropyl aminoethyl (meth)acrylate, and dibutyl aminoethyl (meth)acrylate. Specific examples of dialkyl (meth)acrylamide include dimethyl methacryl amide. Specific examples of dialkyl aminoalkyl (meth)acrylamide include dimethyl aminopropyl methacrylamide. In polymerization, a polymerizable monomer containing the hydroxy group such as hydroxyethyl (meth)acrylate, hydroxypropyl (meth)acrylate, 2-hydroxybutyl (meth)acrylate, or N-methylol (meth)acrylamide can be used together.

The amount of charge control agent used is not particularly limited within the scope consistent with the object of the present disclosure. Typically, the amount of charge control agent used is, relative to the total mass of the toner core particle, preferably 0.1 mass% or more but 10 mass% or less. Using too small an amount of charge control agent makes it difficult to stably charge the toner with a predetermined polarity. This can lead to a lower-than-expected value in the image density of the formed image and make it difficult to maintain satisfactory image density for a long period. Also, the charge control agent is then difficult to disperse evenly, and this tends to cause fogging in the formed image and contamination of a latent image carrying member with toner components. Using too large an amount of charge control agent can lead to poorer resistance to environment and this tends to cause image faults in the formed image due to insufficient charging under high temperature and high humidity, contamination of a latent image carrying member with toner components, and the like.

### (Shell Material)

If the shell layer is formed on the surface of the toner core particle, the shell layer is formed of, for example, a vinyl-based resin. As the vinyl-based resin used to form the shell layer, a resin containing a charge control resin is used. With the shell layer formed of a resin containing a charge control resin, when images are formed for a long period in various environments such as a high-temperature high-humidity environment and a low-temperature low-humidity environment, it is possible to charge the toner with the desired charge amount and to form images with the desired density.

Preferably, the vinyl-based resin is a styrene-acrylic acid-based resin containing a styrene-based monomer and one or more types of acrylic acid-based monomers. The styrene-acrylic acid-based resin has strong hydrophobicity and tends to be easy to charge positively. It is considered that forming the shell layer of styrene-acrylic acid-based resin gives it a higher affinity for the resin fine particles formed of silicone modified acrylic resin that are attached as an external additive to the toner base particle, suppressing the coming-off of the resin fine particles from the shell layer.

The amount of vinyl-based resin used is not particularly limited within the scope consistent with the object of the present disclosure. Typically, the amount of vinyl-based resin used is preferably, for 100 parts by mass of the toner core particle, 1 part by mass or more but 20 parts by mass or less, and more preferably 3 parts by mass or more but 15 parts by mass or less. Using too small an amount of vinyl-based resin may result in the shell layer failing to coat the entire surface of the toner core particle. If the shell layer fails to coat the entire surface of the toner core particle, the toner tends to agglomerate during storage at high temperature, leading to poor heat-resistant preservation properties. On the other hand, using too large an amount of vinyl-based resin tends to increase the thickness of the shell layer. This makes it difficult to produce toner that excels in fixing properties.

The mass average molecular weight (Mw) of the vinyl-based resin used to form the shell layer is not particularly limited within the scope consistent with the object of the present disclosure. Typically, the mass average molecular weight is preferably 20,000 or more but 1,500,000 or less, and more preferably 200,000 or more but 400,000 or less. The mass average molecular weight (Mw) of the vinyl-based resin can be measured by gel permeation chromatography according to any known method.

A method of polymerizing the monomer (monomeric substance) described above is not particularly limited within the scope consistent with the object of the present disclosure, and thus any of methods such as solution polymerization, bulk polymerization, emulsion polymerization, and suspension polymerization can be selected.

In a case where, as in emulsion polymerization or suspension polymerization, a monomer having an unsaturated bond is addition-polymerized using an aqueous solvent, a surfactant can be used. The surfactant is not particularly limited within the scope consistent with the object of the present disclosure and can be appropriately selected from the group consisting of anionic surfactants, cationic surfactants, and nonionic surfactants. Examples of anionic surfactants include sulfate ester salt-type surfactants, sulfonate salt-type surfactants, phosphate ester salt-type surfactants, and soap. Examples of cationic surfactants include amine salt-type surfactants and quaternary ammonium salt-type surfactants. Examples of nonionic surfactants include polyethylene glycol-type surfactants, alkylphenol-ethylene oxide adduct-type surfactants, and polyhydric alcohol-type surfactants that are a derivative of a polyhydric alcohol such as glycerin, sorbitol, or sorbitan. Among these surfactants, at least one of an anionic surfactant and a nonionic surfactant is preferably used. Of these surfactants, one type can be used singly or two or more can be used in combination.

### (External Additive)

In the toner, the toner base particle can have, as desired, its surface treated with an external additive. The type of external additive is not particularly limited within the scope consistent with the object of the present disclosure and thus can be selected appropriately from external additives known to be used in toner. Specific examples of suitable external additives include inorganic fine particles of silica or a metal oxide or the like such as alumina, titanium oxide, magnesium oxide, zinc oxide, strontium titanate, or barium titanate, or resin fine particles of acrylic resin, silicone modified acrylic resin, or the like. Two or more of these external additives can be used in combination.

The particle size of the external additive is not particularly limited within the scope consistent with the object of the present disclosure. Typically, it is preferably 0.01 µm or more but 1.0 µm or less.

The amount of external additive used is not particularly limited within the scope consistent with the object of the present disclosure. Typically, it is preferably, for the total mass of the toner base particle produced with the shell layer formed on the surface of the toner core particle, 0.1 mass% or more but 10 mass% or less, and more preferably 0.2 mass% or more but 5 mass% or less. Using too small an amount of external additive tends to degrade the hydrophobicity of the toner. This makes the toner susceptible to water molecules in the air in a high-temperature high-humidity environment and tends to cause problems such as a drop in the image density of the formed image resulting from an extreme drop in the charge amount of toner as well as a drop in the fluidity of the toner. On the other hand, using too large an amount of external additive may result in a drop in the image density due to the excessive charging of the toner.

Next, a production method for the toner will be described. The production method for the toner is not particularly limited so long as it can form the toner core particle and the shell layer with predetermined structures. As necessary, using as the toner base particle the toner core particle coated with the shell layer, external addition treatment can be applied to the surface of the toner base particle to attach the external additive to it. As a suitable production method for the toner described above for development of electrostatic latent images, a method for producing the toner core particle, a method for forming the shell layer, and a method for external addition treatment will be described one by one below.

### (Method for Producing Toner Core Particle)

The method for producing the toner core particle is not particularly limited so long as it can satisfactorily disperse any optional components such as a colorant, a release agent, a charge control agent, and a magnetic powder in the binder resin. In one specific example of a suitable method for producing the toner core particle, the binder resin and any components such as a colorant, a release agent, a charge control agent, and a magnetic powder are mixed using a mixer or the like; then the binder resin and the components blended in the binder resin are melted and kneaded using a kneader such as a uniaxial or biaxial extruder; and the cooled kneaded product is pulverized and classified. The average particle size of the toner core particle is not particularly limited within the scope consistent with the object of the present disclosure; in general, it is preferably 5 µm or more but 10 µm or less.

### (Method for Forming Shell Layer)

To form the shell layer, fine particles of vinyl-based resin is attached to the surface of the toner core particle to coat it.

The method will be described more specifically. First, in a mixing apparatus, hydrochloric acid is added to ion-exchange water to prepare an aqueous solvent with weak acidity (e.g., with a pH value selected from the range of three or more but five or less). Subsequently, to the aqueous solvent with the so adjusted pH value, a dispersion liquid (suspension) of fine particles of the vinyl-based resin as a shell material and the toner core particles are added.

Subsequently, while the mixture liquid containing the shell material and the toner core particle mentioned above is stirred, the temperature of the mixture liquid is raised up to a predetermined holding temperature (e.g., a temperature selected from the range of 50°C or more but 90°C or less) at a predetermined rate (e.g., a rate selected from the range of 0.1°C/min or more but 3°C/min or less). Then, the mixture liquid is, while being stirred, held at the predetermined holding temperature for a predetermined time (e.g., a length of time selected from the range of 30 minutes or more but 4 hours or less). It is considered that, while the temperature of the mixture liquid is held high, a reaction (fixation of the shell layer) proceeds between the toner core particle and the shell material. The shell material binds to the toner core particle to form the shell layer. The formation of the shell layer on the surface of the toner core particle in the mixture liquid yields a dispersion liquid of toner base particles.

As described above, attaching fine particles of vinyl-based resin, which is hydrophobic, to the surface of the toner core particle in the mixture liquid and heating the mixture liquid permits the fine particles of vinyl-based resin to melt and form a film. Instead, the fine particles of vinyl-based resin can be heated in a drying step or subjected to physical impact in an external addition step, to promote their film formation.

After the shell layer is formed as described above, the dispersion liquid of toner base particles is neutralized using, for example, sodium hydroxide. Subsequently, the dispersion liquid of toner base particles is cooled to, for example, normal temperature (about 25°C). Then, the dispersion liquid of toner base particles is filtered using, for example, a Buchner funnel. This separates the toner base particles from the liquid (solid-liquid separation) and yields toner base particles in the form of a wet cake. Next, the obtained toner base particles in the form of a wet cake are washed. The washed toner base particles are then dried. After that, as necessary, using a mixer (e.g., an FM mixer manufactured by NIPPON COKE & ENGINEERING CO., LTD.), the toner base particles and the external additive can be mixed to attach the external additive to the surface of the toner base particles. If a spray drier is used in the drying step, spraying the dispersion liquid of the external additive (e.g., silica particles) to the toner base particles makes it possible to carry out the drying step and the external addition step at the same time. In this way, toner including a large number of toner particles is produced.

The steps involved and their order in the method for producing toner described above can be freely changed depending on the desired configuration or properties of the toner. After the external addition step, the toner can be sieved. Any unnecessary step can be omitted. For example, if a commercially available product can be used as it is as a material, using the commercially available product helps eliminate a step of preparing that material. Likewise, if a reaction to form the shell layer satisfactorily proceeds without the adjustment of the pH value of the mixture liquid, a pH adjusting step can be omitted. If no external additive is attached to the surface of the toner base particle (an external addition step is omitted), the toner base particle corresponds to the toner particle. To produce toner efficiently, it is preferable to form a large number of toner particles at the same time. The toner particles produced at the same time are considered to share substantially the same configuration.

### (Method for External Addition Treatment)

The method for treatment of the toner base particle with the external additive is not particularly limited; the toner base particle can be treated by any known method. Specifically, the toner base particle is treated with the external additive using a mixer such as a Henschel mixer or a Nauta mixer under treatment conditions adjusted such that the particles of the external additive do not sink in the toner base particle.

The two-component developer that uses the toner described above and the magnetic carrier according to the present disclosure excels in fixing properties and heat-resistant preservation properties. In cases where images are formed for a long period in various environments including a high-temperature high-humidity environment and a low-temperature low-humidity environment, the toner can be electrostatically charged to a desired charge amount. Thus, the images can be formed with the desired density. Accordingly, the magnetic carrier according to the present disclosure can be suitably used in a variety of image forming apparatuses of two-component development type. Now, the effects of the present disclosure will be described more specifically by way of examples. The present disclosure is not limited in any way by those examples.

### EXAMPLES

### [Production Example 1]

### (Production of Toner Core Particle)

As the binder resin, for 100 mass parts of polyester resin (XPE258, manufactured by Mitsui Chemicals, Inc.), 5 mass parts of polypropylene wax (660P, manufactured by SANYO CHEMICAL INDUSTRIAL CO. LTD.), 5 mass parts of carbon black (REGAL330R, manufactured by Cabot Corporation.), and 1 mass part of charge control agent (BONTRON P-51, manufactured by ORIENT CHEMICAL INDUSTRIES CO., LTD.) were weighed. All these were mixed using a Henschel mixer (FM-10B, manufactured by NIPPON COKE & ENGINEERING CO., LTD.), and then the mixture was melted and kneaded using a biaxial extruder. The obtained kneaded product was cooled, and was then pulverized and classified to obtain toner core particles with a volume average particle size of 7 µm. The volume average particle size was measured using a Coulter Counter Multisizer 3 (manufactured by Beckman Coulter, Inc.).

### [Production Example 2]

### (Production of Toner)

To the toner core particles obtained in production example 1, relative to their total mass, 1.0 mass% of titanium oxide (EC-100, manufactured by Titan Kogyo, Ltd.) and 0.7 mass% of hydrophobic silica (RA-200H, manufactured by NIPPON AEROSIL CO., LTD.) treated with aminosilane, were added. The mixture was then mixed for five minutes at a rotation rate of 3500 rpm using a Henschel mixer (FM-10B, manufactured by NIPPON COKE & ENGINEERING CO., LTD.) to obtain toner for development of electrostatic latent images.

### [Production Example 3]

### (Production of Magnetic Carrier)

### (3-1. Production of Carrier Core)

As magnetic particles, non-coat ferrite particles (F-350, manufactured by Powdertech Co., Ltd., with a volume average primary particle size of 35 µm) were stirred using a multipurpose mixer (manufactured by NIPPON COKE & ENGINEERING CO., LTD., with, as a tank, a CP tank and, as a stirring blade, one for a CP tank) (smoothing treatment) with the rotation rate and stirring time adjusted to obtain carrier cores C-1 to C-8 that had different amounts of fine particles present on them. Note that the carrier core C-1 was untreated (i.e., it was not subjected to the smoothing treatment using a mixer).

The obtained carrier cores C-1 to C-8 were measured using a laser diffraction grain size distribution analyzer (SYNC, manufactured by MicrotracBEL Corp.) (wet measurements) to measure the amount of fine particles present on the carrier core. Table 1 shows the amount of fine particles present on carrier cores C-1 to C-8 along with the rotation rate of the mixer and the stirring time. Figs. 5 to 10 show photographs (at 500 times and 1000 times magnifications) of carrier cores C-1, C-4, and C-6 on a scanning electron microscope (SEM).

**[Table 1]**

| Carrier Core | Mixer Rotation Rate [rpm] | Stirring Time [min] | Amount of Fine Particles Present [%] |
|---|---|---|---|
| C-1 | - | - | 0.1 |
| C-2 | 2500 | 10 | 0.6 |
| C-3 | 5000 | 5 | 1.8 |
| C-4 | 5000 | 10 | 2.0 |
| C-5 | 7500 | 5 | 4.0 |
| C-6 | 7500 | 10 | 10.0 |
| C-7 | 7500 | 20 | 20.0 |
| C-8 | 10000 | 10 | 25.0 |

### (3-2. Formation of Resin Coat Layer)

The solid content of the silicone-based resin (SR-2411, manufactured by Toray Dow Corning Silicone Corp., the solid content: 20 mass%) was mixed with 15 mass% of aminosilane, and these were dissolved in a toluene to obtain a resin coat layer forming solution. The obtained resin coat layer forming solution was sprayed-coated to carrier core C-4 obtained as described in 3-1 above using a fluidized bed-coating machine (manufactured by Powrex Corporation). Then, in the fluidized bed, heat treatment was performed for 3 hours at 250 °C to set the resin to obtain carrier of Practical Example 1 of the present disclosure.

Carrier of Practical Example 2 was obtained in a manner similar to that of Practical Example 1 except that carrier core C-5 was used instead of carrier core C-4.

Carrier of Practical Example 3 was obtained in a manner similar to that of Practical Example 1 except that carrier core C-6 was used instead of carrier core C-4.

Carrier of Practical Example 4 was obtained in a manner similar to that of Practical Example 1 except that carrier core C-7 was used instead of carrier core C-4.

Carrier of Comparative Example 1 was obtained in a manner similar to that of Practical Example 1 except that carrier core C-1 was used instead of carrier core C-4.

Carrier of Comparative Example 2 was obtained in a manner similar to that of Practical Example 1 except that carrier core C-2 was used instead of carrier core C-4.

Carrier of Comparative Example 3 was obtained in a manner similar to that of Practical Example 1 except that carrier core C-3 was used instead of carrier core C-4.

Carrier of Comparative Example 4 was obtained in a manner similar to that of Practical Example 1 except that carrier core C-8 was used instead of carrier core C-4.

[Evaluation of Image Fogging of Two-Component Developer]

The toner obtained in production example 2 and each of the carriers of Practical Examples 1 to 4 and of Comparative Examples 1 to 4 obtained in production example 3 were blended so that the product had a toner concentration of 7 mass% (i.e., so that the amount of toner added was 7 mass parts for 100 mass parts, that is, the total amount, of toner and carrier) and the product was stirred and mixed for 30 minutes using a rocking mixer to obtain two-component developers respectively containing the carriers of Practical Examples 1 to 4 and of Comparative Examples 1 to 4.

A development device in an evaluation machine (TASKalfa 2553ci, manufactured by KYOCERA Document Solutions Inc.) was loaded with the two-component developer obtained as described above. In a normal-temperature and normal-humidity environment (NN environment, temperature: 25 °C, humidity; 50%), continuous printing was performed on 100,000 sheets at a test image coverage rate of 5%. Then the evaluation machine was moved to be left to stand still in a high-temperature high-humidity environment (referred to as HH environment where the temperature was 32.5°C, and the humidity was 80%) for one day. After that, initial images were acquired in the HH environment.

The fogging density (FD) in a blank part of the images on the print results was measured using a reflection density sensor (SpectroEye, manufactured by X-Rite, Incorporated) at the following times: at an initial stage in the NN environment (at the start of printing), after durability printing on 100,000 sheets, and at an initial stage in the HH environment. The fogging density (FD) was calculated according to formula (1) below. FD = (reflection density in blank part of printed sheet) - (reflection density on unprinted sheet)

The evaluation criteria for image fogging were as follows:
VERY GOOD: FD ≤ 0.005 (particularly low FD, very good print result)
GOOD: 0.005 < FD ≤ 0.010 (low FD, good print result)
POOR: FD > 0.010 (very high FD, poor image quality)

Table 2 shows the results of evaluation of image fogging with each of the two-component developers respectively containing the carriers of Practical Examples 1 to 4 and of Comparative Examples 1 to 4.

**[Table 2]**

| | Fogging Density [FD] | | | Evaluation |
|---|---|---|---|---|
| | Initial Stage in NN Environment | After Durability Printing on 100k Sheets | Initial Stage in HH Environment | |
| Practical Example 1 | 0.002 | 0.003 | 0.008 | GOOD |
| Practical Example 2 | 0.002 | 0.005 | 0.009 | GOOD |
| Practical Example 3 | 0.001 | 0.004 | 0.005 | VERY GOOD |
| Practical Example 4 | 0.002 | 0.003 | 0.004 | VERY GOOD |
| Comparative Example 1 | 0.003 | 0.006 | 0.020 | POOR |
| Comparative Example 2 | 0.002 | 0.005 | 0.015 | POOR |
| Comparative Example 3 | 0.003 | 0.006 | 0.011 | POOR |
| Comparative Example 4 | 0.003 | 0.003 | 0.004 | POOR (*) |

| | | | | |
|---|---|---|---|---|
| * Many cracked carrier cores caused carrier development. | | | | |

Table 2 reveals the following. The carriers of Practical Examples 1 to 4, which used carrier cores C-4 to C-7 in which the amount of fine particles present on their surface was 2% or more but 20% or less, were very good or good in image fogging after standing-still for one day in a high-temperature high-humidity environment. In particular, the carriers of Practical Examples 3 and 4, which used carrier cores C-6 and C-7 in which the amounts of fine particles present on their surfaces were 10 % and 20%, respectively, were very good in image fogging.

In contrast, the carriers of Comparative Examples 1 to 3, which used carrier cores C-1 to C-3 in which the amount of fine particles present on their surface was less than 2% were poor in image fogging after standing-still for one day in a high-temperature high-humidity environment. With the carrier of Comparative Example 4, which used carrier core C-8 in which the amount of fine particles present on its surface was 25%, many cracked carrier cores caused carrier development and hence problems in quality and thus the overall quality was judged to be poor.

The above results confirm that using magnetic carrier obtained by performing smoothing treatment on a carrier core to grind off elevated parts of the carrier core to produce fine particles such that the amount of fine particles present on the surface of the carrier core is 2% or more but 20% or less and then coating the surface of the carrier core with a resin coat layer yields two-development developer that helps prevent image fogging under a high-temperature high-humidity environment.

The present disclosure finds application in magnetic carrier that electrostatically charges toner by friction with it. Based on the present disclosure, it is possible to provide magnetic carrier for use in electrophotography and two-component developer that excel in charging ability and charge keeping ability even in a high-temperature high-humidity environment and that permit development with high durability and high image quality.

The above embodiments of the invention as well as the appended claims and figures show multiple characterizing features of the invention in specific combinations. The skilled person will easily be able to consider further combinations or sub-combinations of these features in order to adapt the invention as defined in the claims to his specific needs.

## Claims

1. Magnetic carrier comprising:
a carrier core (1); and
a resin coat layer (5) that coats a surface of the carrier core (1),
the magnetic carrier being capable of electrostatically charging toner by friction,
**characterized in that**
the carrier core (1) has, in a depressed part (3) in the surface thereof, fine particles (4) of which a volume average primary particle size is 1 µm or less, and an amount of the fine particles (4) present on the surface of the carrier core (1) is, on a number basis when a particle distribution of the carrier core (1) is measured, 2% or more but 20% or less.

2. The magnetic carrier according to claim 1, **characterized in that**
a volume average primary particle size of the carrier core (1) is 30 µm or more but 65 µm or less.

3. The magnetic carrier according to claim 1, **characterized in that**
the fine particles (4) have a same composition as the carrier core (1).

4. The magnetic carrier according to claim 1, **characterized in that**
the fine particles (4) are produced by applying an external force to the carrier core (1).

5. The magnetic carrier according to claim 1, **characterized in that**
the resin coat layer (5) is formed of silicone-based resin.

6. Two-component developer comprising:
the magnetic carrier according to claim 1; and
toner that is electrostatically charged positively by friction with the magnetic carrier.

7. A method for producing magnetic carrier comprising:
a carrier core (1); and
a resin coat layer (5) that coats a surface of the carrier core (1), and
the magnetic carrier being capable of electrostatically charging toner by friction,
the method comprising:
a smoothing step of stirring the carrier core (1) using a mixer to grind off elevated parts (2) on the surface of the carrier core (1) so as to produce fine particles (4) of which a volume average particle size is 1 µm or less;
an application step of, after the smoothing step, applying a resin coat layer forming solution to the surface of the carrier core (1); and
a heating step of, after the application step, heating the carrier core (1) to form the resin coat layer (5) on the surface of the carrier core (1).

8. The method according to claim 7, **characterized in that**,
an amount of the fine particles (4) present on the surface of the carrier core (1) is adjusted to be, on a number basis when a particle distribution of the carrier core (1) is measured, 2% or more but 20% or less by controlling a rotation rate and a stirring time of the mixer in the smoothing step.
